# EUROPEAN PATENT APPLICATION

(11) **EP 4 696 823 A1**
(43) Date of publication of application: **18.02.2026**
(21) Application number: 24788618.7
(22) Date of filing: 02.04.2024
(51) Int. Cl.: D01F 6/62, D02G 3/04

(54) **POLYTRIMETHYLENE TEREPHTHALATE FIBER, METHOD FOR PRODUCING SAME, AIR-MIXED FILAMENT YARN CONTAINING SAID POLYTRIMETHYLENE TEREPHTHALATE FIBER, AND FABRIC COMPOSED THEREOF**

(30) Priority: 11.04.2023 JP 2023064016; 11.04.2023 JP 2023064017
(71) Applicant: TEIJIN FRONTIER CO., LTD., Osaka-shi, Osaka 530-0005 (JP)
(72) Inventor: YONEDA, Hiroyuki, Osaka-shi, Osaka 530-0005 (JP); OGATA, Nobuaki, Osaka-shi, Osaka 530-0005 (JP); NAGAO, Hideharu, Osaka-shi, Osaka 530-0005 (JP)
(74) Representative: Carpmaels & Ransford LLP
(86) International application number: PCT/JP2024/013587
(87) International publication number: WO 2024/214591

(57) **Abstract**

An object of the present invention is to provide a low-shrinkage fiber substantially composed of polytrimethylene terephthalate, which can be used to produce a raw yarn for cloth having a small shrinkage rate on heating and a soft hand, and a method for producing the same, an air-jet commingled yarn containing the polytrimethylene terephthalate fiber, and cloth composed thereof. In the present invention, there is provided a polytrimethylene terephthalate fiber composed of 90 mol% or more of a trimethylene terephthalate repeating unit. The polytrimethylene terephthalate fiber has a boiling water shrinkage rate of 5% or less and a modulus at an elongation of 20% of 5 cN/dtex or less.

## Description

### Technical Field

The present invention relates to a fiber substantially composed of polytrimethylene terephthalate, which can be used to produce a raw yarn for cloth having a small shrinkage rate on heating and a soft hand, and a method for producing the same, an air-jet commingled yarn containing the polytrimethylene terephthalate fiber, and cloth composed thereof.

### Background Art

Polytrimethylene terephthalate (hereinafter, may be referred to as PPT) has properties similar to those of polyamide, such as excellent elastic recovery and dyeability, and properties similar to those of polyethylene terephthalate, such as light resistance, heat setting, dimensional stability, and low water absorption, and thus has been proposed to be used in many fields of a BCF carpet, a brush, and the like by taking advantage of these properties (for example, JPH09-3724A, JPH08-173244A, and JPH05-262862A). Further, a polytrimethylene terephthalate fiber has a low Young's modulus, so that it is said that a product having a soft hand can be obtained.

As a method for producing a polytrimethylene terephthalate fiber, a method has been proposed in which an undrawn yarn obtained by melt spinning at 300 m/min to 4000 m/min is hot drawn in one stage or multiple stages at a temperature equal to or higher than a glass transition temperature of the undrawn yarn, either after being wound up or continuously without being wound up. As spinning and drawing conditions therefor, for example, JP2001-207329A (PTL 1) discloses a method in which a polytrimethylene terephthalate polymer having intrinsic viscosity [η] of 0.7 or more is taken off at a spinning speed of 3000 m/min, and then drawn at 70°C without intermediate winding, followed immediately by a relaxation heat treatment with a relaxation rate of 6% to 20%.

However, although the polytrimethylene terephthalate fiber proposed in related art certainly has a Young's modulus lower than that of a polyethylene terephthalate fiber, when the polytrimethylene terephthalate fiber is made into cloth, these properties are not fully exhibited, and cloth that is fully satisfactory in terms of softness has not yet been obtained.

On the other hand, JP2001-348729A (PTL 2) discloses that a polytrimethylene terephthalate fiber having a soft hand can be obtained by winding at a spinning speed of 4500 m/min or more. In the method, although soft cloth is obtained, during yarn winding, elastic deformation of the yarn causes winding tension, resulting in poor winding shape and crushed wound paper tubes. Further, since the spinning speed is high, yarn breakage is likely to occur, and stable yarn production is difficult.

### Citation List

### Patent Literature

PTL 1: JP2001-207329A
PTL 2: JP2001-348729A

### Summary of Invention

### Technical Problem

The present invention has been made in view of the above background, and an object of the present invention is to provide a low-shrinkage fiber substantially composed of polytrimethylene terephthalate, which can be used to produce a raw yarn for cloth having a small shrinkage rate on heating and a soft hand, and a method for producing the same, an air-jet commingled yarn containing the polytrimethylene terephthalate fiber, and cloth composed thereof.

### Solution to Problem

As a result of intensive studies to solve the above problems, the present inventors have found that a desired polytrimethylene terephthalate fiber can be obtained by controlling a boiling water shrinkage rate (hereinafter, may be referred to as boiling water shrinkage rate) of a fiber substantially composed of polytrimethylene terephthalate and a modulus of the polytrimethylene terephthalate fiber at an elongation of 20% within a range different from that of a so-called partially oriented yarn or high-speed spinning yarn described in the above citation list, and have completed the present invention.

Thus, the present invention provides
1. a polytrimethylene terephthalate fiber including: 90 mol% or more of a trimethylene terephthalate repeating unit, in which the polytrimethylene terephthalate fiber has a boiling water shrinkage rate of 5% or less and a modulus at an elongation of 20% of 5 cN/dtex or less
2. the polytrimethylene terephthalate fiber according to the above 1, in which the polytrimethylene terephthalate fiber has a birefringence Δn of 0.040 or more and a specific gravity of 1.350 or less
3. the polytrimethylene terephthalate fiber according to the above 1 or 2, in which the polytrimethylene terephthalate fiber has a thermal stress peak at 50°C to 100°C and a thermal stress peak value of 0.2 cN/dtex or less
4. the polytrimethylene terephthalate fiber according to the above 1 or 2, in which the polytrimethylene terephthalate fiber has breaking strength of 1.5 cN/dtex to 3.5 cN/dtex and a breaking elongation of 30% to 100%
5. a method for producing a polytrimethylene terephthalate fiber, the method including: melting and solidifying polytrimethylene terephthalate composed of 90 mol% or more of a trimethylene terephthalate repeating unit; winding up the polytrimethylene terephthalate at a winding speed of 1000 m/min or more; drawing the polytrimethylene terephthalate to 1.1 times or more at a temperature equal to or lower than a glass transition point of the polytrimethylene terephthalate; and shrinking the fiber at a ratio of 0.5 times to 0.9 times while heating
6. an air-jet commingled yarn including: the polytrimethylene terephthalate fiber according to any one of the above 1 to 4; and a polyester fiber
7. the air-jet commingled yarn according to the above 6, including the polyester fiber has a boiling water shrinkage rate of 7% to 50%
8. the air-jet commingled yarn according to the above 6 or 7, further including: a modified cross-section fiber
9. a core-sheath type air-jet commingled yarn obtained by heat-treating the air-jet commingled yarn according to claim 6, the core-sheath type air-jet commingled yarn including: a core yarn; and a sheath yarn, in which the air-jet commingled yarn has a total fineness of 30 dtex to 400 dtex, the core yarn is composed of a polyester fiber, the sheath yarn is composed of a polytrimethylene terephthalate fiber having a single fiber fineness of 0.3 dtex to 10 dtex, and a yarn length difference between the core yarn and the sheath yarn is 5% or more, as defined by the following method,
   (method for measuring yarn length difference)
   the core-sheath type air-jet commingled yarn is treated in boiling water, then cut to a length of 5 cm under a load of 0.1 cN (0.098 g) × total fineness (dtex) of the core-sheath type air-jet commingled yarn, a polyester fiber A (single fiber) and a polytrimethylene terephthalate fiber B (single fiber) are taken out from the cut core-sheath type air-jet commingled yarn, a length of each is measured under a load of 0.1 cN (0.098 g) × single fiber fineness (dtex) thereof, and the yarn length difference (%) is calculated by the following formula:$Yarn length difference \left(%\right) = \left(LB - LA\right) / LA \times 100$ where LA is a yarn length (cm) of the polyester fiber of the core yarn, and LB is a yarn length (cm) of the polytrimethylene terephthalate fiber of the sheath yarn
10. the core-sheath type air-jet commingled yarn according to the above 9, in which a weight ratio of the sheath yarn to a total weight of the core-sheath type air-jet commingled yarn is 50% to 90%
11. the core-sheath type air-jet commingled yarn according to claim 9 or 10, further including: a modified cross-section fiber
12. cloth including: the air-jet commingled yarn according to any one of the above 6 to 8
13. cloth including: the core-sheath type air-jet commingled yarn according to any one of the above 9 to 11.

### Advantageous Effects of Invention

According to the present invention, a low-shrinkage fiber substantially composed of polytrimethylene terephthalate, which can be used to produce a raw yarn for cloth having a small shrinkage rate on heating and a soft hand, and a method for producing the same, an air-jet commingled yarn containing the polytrimethylene terephthalate fiber, and cloth composed thereof can be provided.

### Brief Description of Drawings

[FIG. 1] FIG. 1 is a schematic view illustrating an example of a modification degree in a modified cross-section fiber used in the present invention.
[FIG. 2] FIG. 2 is a schematic view illustrating an example of flatness of a flat cross-section fiber used in the present invention.

### Description of Embodiments

Hereinafter, the present invention will be described in detail.

### (1) Polymer Raw Material

A polymer used in the present invention is polytrimethylene terephthalate (hereinafter may be referred to as PTT) composed of 90 mol% or more of a trimethylene terephthalate repeating unit. Here, the PTT is a polyester containing terephthalic acid as an acid component and trimethylene glycol (also known as 1,3-propanediol) as a diol component. The PTT may contain 10 mol% or less of other copolymerization components.

Examples of such copolymerization components include ester-forming monomers such as 5-sodium sulfoisophthalic acid, 5-potassium sulfoisophthalic acid, 3,5-dicarboxylic acid benzenesulfonic acid tetrabutylphosphonium salt, 3,5-dicarboxylic acid benzenesulfonic acid tributylmethylphosphonium salt, 1,4-butanediol, neopentyl glycol, 1,6-hexamethylene glycol, 1,4-cyclohexanediol, 1,4-cyclohexanedimethanol, adipic acid, dodecanedioic acid, and 1,4-cyclohexanedicarboxylic acid.

If necessary, the PTT may be copolymerized with or mixed with various additives such as a matting agent, a heat stabilizer, an antifoaming agent, a tinting agent, a flame retardant, an antioxidant, an ultraviolet absorber, an infrared absorber, a crystal nucleating agent, and a fluorescent whitening agent.

In the polytrimethylene terephthalate polymer used in the present invention, intrinsic viscosity [η] is preferably 0.5 to 1.6, and more preferably 0.6 to 1.5. The intrinsic viscosity [η] is still more preferably 0.7 to 1.4.

It is not preferable that the intrinsic viscosity is less than 0.5, since it may be difficult to develop strength due to the molecular weight of the polymer being too low. On the other hand, it is not preferable that the intrinsic viscosity exceeds 1.6, since the low viscosity polytrimethylene terephthalate may suffer from impaired spinnability due to poor fluidity, which can cause yarn breakage during spinning.

### (2) Polytrimethylene Terephthalate Fiber

The polytrimethylene terephthalate fiber of the present invention is less deformed by a hot water treatment, and therefore when made into cloth, the yarn shrinks little and has a soft hand. Since a modulus of the polytrimethylene terephthalate fiber after a primary yield point in a tensile strength and elongation measurement is low as a characteristic of the polytrimethylene terephthalate fiber, cloth made from the polytrimethylene terephthalate fiber has enhanced drapability with softness compared to an ordinary polytrimethylene terephthalate fiber.

As for yarn properties of such a polytrimethylene terephthalate fiber, a boiling water shrinkage rate (hereinafter may be referred to as boiling water shrinkage rate) of the polytrimethylene terephthalate fiber in the present application is required to be 5% or less, and is preferably 4% or less, and more preferably 3% or less. When the boiling water shrinkage rate is more than 5%, the cloth becomes stiff due to yarn shrinkage caused by thermal shrinkage.

In the polytrimethylene terephthalate fiber of the present invention, a modulus at an elongation of 20% is required to be 5 cN/dtex or less, and is preferably 4 cN/dtex or less, and more preferably 3 cN/dtex or less. When the modulus at an elongation of 20% is greater than 5 cN/dtex, the cloth becomes stiff due to subsequent dyeing and other processing.

Further, a birefringence Δn of the polytrimethylene terephthalate fiber of the present invention is preferably 0.040 or more and 0.08 or less. More preferably, the birefringence Δn is 0.045 or more and 0.075 or less, and even more preferably, the birefringence Δn is 0.050 or more and 0.070 or less. It is not preferable that the birefringence Δn is less than 0.040, since the yarn strength is small and the cloth is elongated by an external force, which makes it difficult to maintain the form.

Further, a specific gravity as an alternative index indicating crystallinity of the polytrimethylene terephthalate fiber of the present invention is preferably 1.350 or less, and more preferably 1.319 or more and 1.350 or less. When the specific gravity is less than 1.319, the yarn becomes brittle during draw-twisting, and yarn breakage frequently occurs, and the draw-twisting becomes difficult. On the other hand, it is not preferable that the specific gravity is larger than 1.350, since a large amount of fluff occurs.

A thermal stress peak of the polytrimethylene terephthalate fiber of the present invention is preferably present at 50°C to 100°C. It is not preferable the peak is present at a temperature lower than 50°C, since the heat resistance decreases. It is not preferable that the peak is present at a temperature higher than 100°C, since the crystallinity becomes too high, and the drapability with softness is lost.

Further, a thermal stress peak value of the polytrimethylene terephthalate fiber of the present invention is preferably 0.2 cN/dtex or less. It is not preferable that the thermal stress peak value is larger than 0.2 cN/dtex, since deformation due to the hot water treatment such as dyeing becomes large, and thus, when made into cloth, the yarn shrinks and develops a stiff hand.

Breaking strength of the polytrimethylene terephthalate fiber of the present invention is 1.5 cN/dtex or more to 3.5 cN/dtex, preferably 1.7 cN/dtex to 3.3 cN/dtex, and more preferably 2.0 cN/dtex to 3.0 cN/dtex.

It is not preferable that the breaking strength of the polytrimethylene terephthalate fiber is less than 1.5 cN/dtex, durability of the product is reduced. On the other hand, it is not preferable that the breaking strength of the polytrimethylene terephthalate fiber is larger than 3.5 cN/dtex, since the crystallinity becomes too high and the drapability with softness is lost.

A breaking elongation of the polytrimethylene terephthalate fiber is preferably 30% to 100%. It is not preferable that the breaking elongation of the polytrimethylene terephthalate fiber is less than 30%, since the crystallinity becomes too high and the drapability with softness is lost. On the other hand, it is not preferable that the breaking elongation of the polytrimethylene terephthalate fiber is larger than 100%, since the fiber is elongated when a load is applied to the fiber, and dimensional stability is not excellent.

### (3) Method for Producing Polytrimethylene Terephthalate Fiber

The polytrimethylene terephthalate fiber as described above can be produced, for example, by the following production method.

First, polytrimethylene terephthalate composed of 90 mol% or more of a trimethylene terephthalate repeating unit is melted and solidified, then wound up at a winding speed of 1000 m/min or more, subsequently heated with a heating roller at a glass transition point of the polytrimethylene terephthalate ±20°C, subsequently drawn to 1.0 time to 2.0 times, further wound around a heating roller at 50°C to 150°C, and then temporarily wound into a cheese-shaped package at a speed of 2000 m/min to 4800 m/min.

The polytrimethylene terephthalate fiber having a breaking elongation of 50% to 200% that is thus wound into a cheese-shaped package is drawn to 1.1 times or more at a temperature equal to or lower than the glass transition point of the polytrimethylene terephthalate, and then the fiber is shrunk at a ratio of 0.5 times to 0.9 times while being heated, thereby obtaining a polytrimethylene terephthalate fiber that can be made into cloth having little thermal shrinkage and a soft hand.

In this case, a total draw ratio, which is expressed as a product of a draw ratio at a temperature equal to or lower than the glass transition point and a shrinkage ratio while heating, is preferably 0.9 times to 1.25 times, and more preferably 0.95 times to 1.20 times. It is not preferable that the total draw ratio is less than 0.90 times, since the yarn may be loosened and running of the yarn during drawing may not be stable, which may lead to yarn breakage. On the other hand, it is not preferable that the total draw ratio is larger than 1.25 times, since the shrinkage rate of the yarn becomes too high, and the cloth made from the yarn may not have a soft hand.

The melted and solidified polytrimethylene terephthalate fiber having a breaking elongation of 50% to 200% can also be produced, for example, by winding at a winding speed of spinning speed 1000 m/min or more and subsequently drawing at a low ratio of 1.0 time to 2.0 times at a temperature of the glass transition point of polytrimethylene terephthalate ± 20°C.

The polytrimethylene terephthalate fiber can also be produced by winding around a heating roller at a spinning speed of 4000 m/min or more and then winding up with a winder. Among these methods, there is no problem in heating with the heating roller at 50°C to 150°C before winding, in order to prevent winding tension when the polytrimethylene terephthalate fiber is directly wound with the winder.

The breaking elongation of the high-elongation polytrimethylene terephthalate fiber thus obtained is preferably 50% to 200% or more. The breaking elongation is more preferably 60% to 190%, and still more preferably 70% to 180%.

It is not preferable that the breaking elongation of the high-elongation polytrimethylene terephthalate fiber is less than 50%, since crystallization of the fiber becomes high, and cloth having a soft hand cannot be obtained. On the other hand, it is not preferable that the breaking elongation is more than 200%, since the crystallization does not proceed when drawn at a temperature equal to or lower than the glass transition point, the strength is significantly low, and the durability is reduced when made into cloth.

Subsequently, the melted and solidified polytrimethylene terephthalate fiber is drawn to 1.1 times or more, preferably 1.2 times or more, and more preferably 1.3 times or more at a temperature equal to or lower than the glass transition point of polytrimethylene terephthalate, preferably at a temperature equal to or lower than the glass transition point -5°C, and more preferably at a temperature equal to or lower than the glass transition point -10°C.

At this time, it is not preferable that drawing is performed at a temperature higher than the glass transition point, since the crystallinity increases, and cloth having a soft hand cannot be obtained. On the other hand, it is not preferable that drawing is performed at a ratio lower than 1.1 times, since the durability is reduced when made into cloth.

Since the drawn fiber is less crystalline and shows a high degree of polymer orientation, the dimensional stability by heat is low, and thus the dimensional stability and durability are improved by shrinking the fiber at a ratio of 0.5 times or more and 0.9 times or less while heating.

At this time, it is not preferable that the shrinkage of the fiber is less than 0.5 times, since orientation crystallinity of the obtained polytrimethylene terephthalate fiber becomes too low, and the durability is reduced when made into cloth. On the other hand, it is not preferable that the shrinkage of the fiber is more than 0.9 times, since the crystallinity becomes high, and the cloth having a soft hand cannot be obtained.

### (4) Polyester Fiber (for Core Yarn)

In the present invention, the above polytrimethylene terephthalate fiber and a polyester fiber are commingled by air-jet texturing to obtain an air-jet commingled yarn.

Preferred examples of the polyester fiber used in this case include fibers spun and drawn by a common method, such as a polytrimethylene terephthalate (PTT) fiber, a polyethylene terephthalate (PET) fiber, a side-by-side type or eccentric core-sheath type conjugate fiber of polytrimethylene terephthalate and polyethylene terephthalate, a side-by-side type or eccentric core-sheath type conjugate fiber of polytrimethylene terephthalate and polytrimethylene terephthalate, and a side-by-side type or eccentric core-sheath type conjugate fiber of polyethylene terephthalate and polyethylene terephthalate. In addition, additives such as an antistatic agent, a flame retardant, a heat-resistant agent, a weathering agent, and titanium oxide may be added.

A boiling water shrinkage rate of such a polyester fiber is preferably 7% to 50% in order to increase a yarn length difference between the core yarn and the sheath yarn by applying a heat treatment or the like to the air-jet commingled yarn.

### (5) Method for Producing Air-jet Commingled Yarn

Next, the polytrimethylene terephthalate fiber as a yarn for sheath yarn and the polyester fiber as a yarn for core yarn are aligned, entangled (preferably 30/m to 150/m) by air-jet texturing (interlace or Taslan (registered trademark)), and then taken up with a roller to obtain an air-jet commingled yarn. An overfeed rate during air-jet intermingling is preferably 0.5% to 2%.

Further, the air-jet commingled yarn of the present invention may contain a modified cross-section fiber other than a round cross-section fiber. For example, the air-jet commingled yarn may be composed of a modified cross-section fiber such as a cross-shaped cross-section fiber, a triangular cross-section fiber, or a star cross-section fiber, and in this way, a unique hand can be obtained. Here, as illustrated in FIG. 1, a modification degree of the modified cross-section fiber is a value obtained by measuring a maximum inscribed circle diameter r and a minimum circumscribed circle diameter R of the fiber cross section and calculating the modification degree by R/r, and the value of the modification degree = R/r is preferably 1.15 to 10.0, and more preferably 1.2 to 10.0. When the modification degree is less than 1.15, a difference from the round cross section may be small. When the modification degree exceeds 10.0, a difference in orientation between an outer side and an inner side of a cross-sectional shape of the yarn during spinning becomes large, and the obtained yarn has a lot of fluff and slack, which may be unsuitable for processing.

An example of the modified cross-section fiber is a flat cross-section fiber. It is preferable that the flat cross-section fiber is used, since a unique hand can be obtained. Here, as illustrated in FIG. 2, flatness of the flat cross-section fiber is a value obtained by drawing a rectangle circumscribing the fiber cross section, measuring a long side L and a short side H thereof, and calculating the flatness by L/H, and in the present invention, the value of the flatness = L/H is preferably 2.0 to 10.0. When the flatness is less than 2.0, a difference from the round cross section may be small. When the flatness exceeds 10.0, fluff is likely to be generated during spinning, and stability may be poor.

The thus obtained air-jet commingled yarn can be a core-sheath type air-jet commingled yarn having a large core-sheath yarn length difference, in which a low-shrinkage fiber made of polytrimethylene terephthalate and having a soft hand is used as the sheath yarn.

### (6) Method for Producing Core-sheath Type Air-jet Commingled Yarn

In the present invention, by subjecting the air-jet commingled yarn to a heat treatment such as dyeing, the polytrimethylene terephthalate fiber serves as the sheath yarn and the polyester fiber serves as the core yarn to form a core-sheath type air-jet commingled yarn including the core yarn and the sheath yarn.

In such an air-jet commingled yarn, a single fiber fineness of the sheath yarn is required to be 0.3 dtex to 10 dtex, more preferably 0.5 dtex to 8 dtex, and still more preferably 0.6 dtex to 5 dtex. When the single fiber fineness is larger than 10 dtex, the softness of the cloth may be lost due to the thick single fiber. When the single fiber fineness is smaller than 0.3 dtex, yarn breakage may occur frequently, and the fiber cannot be produced. The number of single fibers (the number of filaments) of the sheath yarn is preferably 20 to 150.

On the other hand, the single fiber fineness of the core yarn is preferably 1.0 dtex to 5.0 dtex. The number of single fibers (the number of filaments) of the core yarn is preferably 12 to 100.

Total fineness of the core-sheath type air-jet commingled yarn of the present invention is required to be 30 dtex to 400 dtex, and is more preferably 50 dtex to 200 dtex. When the total fineness is less than 30 dtex, the total fineness may be too small to perform the air-jet intermingling. On the other hand, when the total fineness is larger than 400 dtex, the softness of the cloth may be lost. The number of single fibers (the number of filaments) is preferably 40 to 400 (more preferably 40 to 200).

In the core-sheath type air-jet commingled yarn, it is important that the yarn length difference between the core yarn and the sheath yarn, as defined below, is 5% or more (more preferably 6% to 40%). When the yarn length difference is less than 5%, sufficient swelling feeling cannot be obtained.

The yarn length difference is calculated by treating the above-described air-jet commingled yarn in boiling water, then cutting the yarn to a length of 5 cm under a load of 0.1 cN (0.098 g) × total fineness (dtex) of the air-jet commingled yarn, taking out the polyester fiber A (single fiber) and the polytrimethylene terephthalate fiber B (single fiber) from the cut air-jet commingled yarn, measuring a length of each under a load of 0.1 cN (0.098 g) × single fiber fineness (dtex) thereof, and calculating the yarn length difference (%) by the following formula.$Yarn length difference \left(%\right) = \left(LB - LA\right) / LA \times 100$ where LA is a yarn length (cm) of the polyester fiber of the core yarn, and LB is a yarn length (cm) of the polytrimethylene terephthalate fiber of the sheath yarn.

In the core-sheath type air-jet commingled yarn of the present invention, the polytrimethylene terephthalate fiber of the sheath yarn is 50% to 90% (more preferably 60% to 80%) in terms of a commingled yarn weight. When a weight ratio of the polytrimethylene terephthalate fiber of the sheath yarn is 50% or less, not only a soft hand cannot be obtained, but also a difference in dyeing between the core yarn and the sheath yarn may be easily observed.

### (7) Method for Producing Cloth Composed of Core-sheath Type Air-jet Commingled Yarn

In the present invention, cloth (greige cloth) is obtained by knitting and weaving using the above-described air-jet commingled yarn, and is then appropriately subjected to dyeing or sweat absorption to obtain cloth as a product. At this time, the yarn length difference between the sheath yarn and the core yarn of the commingled yarn is developed by the heat treatment of dyeing, and cloth composed of the core-sheath type air-jet commingled yarn is obtained.

Here, the cloth may be composed of only the core-sheath type air-jet commingled yarn, or may be composed of the core-sheath type air-jet commingled yarn and other yarns. In this case, the other yarns are not particularly limited, and may be any of a non-crimped yarn, a false twisted crimped yarn, a latent crimped yarn, a spun yarn, and the like.

A structure of the cloth is not particularly limited, and may be either a knitted fabric or a woven fabric. Examples thereof include, but are not limited to, a knitted fabric having a knitting structure such as single jersey, knit-miss, smooth, fleece, knop, plating, Derby rib, and half-gauge, and a woven fabric having a woven structure such as plain weave, twill weave, and satin. The number of layers may be a single layer or a multilayer of two or more layers.

Next, the cloth may be used to produce textile products such as sportswear, outerwear, innerwear, men's clothing, women's clothing, nursing clothing, workwear, a car seat covering material, and bedding. Such cloth and textile products use the above-described air-jet commingled yarn and therefore are excellent in soft hand and swelling.

### [Example]

Hereinafter, Examples and Comparative Examples of the present invention will be described in detail, but the present invention is not limited thereto. Each measurement item in Examples was measured by the following method.

### (1) Intrinsic Viscosity [η]

Intrinsic viscosity [η] was determined using an Ostwald viscometer by extrapolating a ratio ηsp/C of specific viscosity ηsp in o-chlorophenol at 35°C to a concentration C (g/100 ml) to a concentration of zero, according to the following formula (1). $\left[η\right] = lim \left(ηsp/C\right)$ C→0

### (2) Glass Transition Point

A glass transition point was measured from a temperature rise curve obtained by sealing a specified amount of polymer chips in an aluminum sample pan and heating from room temperature to 300°C at a rate of 10°C/min under a nitrogen atmosphere using a DSC.

### (3) Fineness (Fineness of Multifilament Yarn)

Fineness of the multifilament yarn was measured according to JIS-L-1013. A value thereof was divided by the number of single yarns of the multifilament yarn to determine single yarn fineness.

### (4) Boiling Water Shrinkage Rate (BWS)

Based on JIS-L-1013, a fiber is rewound using a sizing reel having a frame circumference of 1.125 m under an initial load of 1/30 g of decitex to make a skein of 20 turns, and a skein length is measured under a load of 1.11 g of decitex. The load was then removed, the skein was immersed in hot water at 100°C for 30 minutes, then taken out and air-dried, and the load was again applied to measure the skein length, and a boiling water shrinkage rate was calculated using the following formula. Boiling water shrinkage rate (%) = {(L0 - L1)/L0} × 100 where L0 is a length (mm) before immersion, and L1 is a length (mm) after immersion.

### (5) Breaking Strength and Breaking Elongation

Based on JIS-L-1013, measurement was performed using a Tensilon, which is a constant speed extension type tensile tester manufactured by Orientec Co., Ltd., at a grip distance of 20 cm and a pulling speed of 20 cm/min.

### (6) Modulus at Elongation of 20%

Based on JIS-L-1013, measurement was performed using a Tensilon, which is a constant speed extension type tensile tester manufactured by Orientec Co., Ltd., at a grip distance of 20 cm and a pulling speed of 20 cm/min. A slope of a tangent line of an SS curve at an elongation of 20% was determined as a modulus at an elongation of 20%.

### (7) Specific Gravity

A specific gravity of a sample was measured based on a sink-float method in JIS-L-1013 8.17.1.

### (8) Birefringence Δn

According to Fiber Handbook-Raw Materials, p. 969 (5th edition, published by Maruzen Co., Ltd. in 1978), a birefringence was determined from a retardation of polarized light observed on a surface of a fiber using an optical microscope and a compensator.

### (9) Temperature at Which Thermal Stress Maximum Value is Present and Thermal Stress Maximum Value

KE-2 manufactured by Kanebo Engineering Co., Ltd. was used. Measurement was performed at an initial load of 0.044 cN/dtex and a heating rate of 100°C/min. The obtained data is plotted with temperature on a horizontal axis and thermal stress on a vertical axis to draw a temperature-thermal stress curve. A temperature and thermal stress at a point where a differential coefficient of the temperature-thermal stress curve changes from positive to negative were determined, and the stress was divided by fineness to determine maximum stress.

### (10) Number of Entanglements

An air-jet textured yarn was cut to a length of 1 m under a load of 8.82 mN/tex (0.1 g/dtex), and after gradual load release, the number of knots was counted following 24-hour relaxation at room temperature, and expressed in piece/m.

### (11) Yarn Length Difference

After skein processing in the same manner as in the above boiling water shrinkage rate, an air-jet commingled yarn was cut to a length of 5 cm under a load of 0.1 cN (0.098 g) × total fineness (dtex) of the air-jet commingled yarn, a polyester fiber A (single fiber) and a polytrimethylene terephthalate fiber B (single fiber) were taken out from the cut air-jet commingled yarn, a length of each was measured under a load of 0.1 cN (0.098 g) × single fiber fineness (dtex) thereof, and a yarn length difference (%) was calculated using the following formula. $Yarn length difference \left(%\right) = \left(LB-LA\right) / LA \times 100$ where LA is a yarn length (cm) of the polyester fiber of the core yarn, and LB is a yarn length (cm) of the polytrimethylene terephthalate fiber of the sheath yarn.

### (12) Hand

A tester touched an air-jet commingled yarn with his or her hand, and evaluated a yarn in three levels of A (swelling and soft), B (normal), and C (poor in swelling or stiff).

### [Example 1]

Dimethyl terephthalate and 1,3-propanediol were charged in a molar ratio of 1:2, and titanium tetrabutoxide equivalent to 0.1% by weight of the dimethyl terephthalate was added, followed by completing a transesterification reaction at a heater temperature of 240°C under normal pressure. Next, 0.1% by weight of titanium tetrabutoxide based on a theoretical polymer amount and 0.5% by weight of titanium dioxide based on the theoretical polymer amount were added, followed by reacting at 270°C for 3 hours.

The obtained polymer was composed of 100 mol% of a trimethylene terephthalate repeating unit and had intrinsic viscosity of 1.0 dl/g. A glass transition point of the obtained polymer was 51°C.

The obtained polymer was dried by a common method to adjust a water content to 50 ppm, then melted at 265°C and extruded through a single-row spinneret having 36 pores with a diameter of 0.27 mm.

The extruded molten multifilament was rapidly cooled by blowing air at a speed of 4.0 m/min to change to a solid multifilament, and then an oil agent containing 60% by weight of octyl stearate, 15% by weight of polyoxyethylene alkyl ether, and 3% by weight of potassium phosphate was applied as a water emulsion finishing agent at a concentration of 10% by weight using a guide nozzle such that an oil agent applied amount was 0.6% by weight with respect to the fiber.

Next, the solid multifilament was wound around a roll heated to 50°C with a peripheral speed of 2100 m/min, then wound around a roll heated to 80°C so as to be drawn to 1.3 times, and then wound at a winding speed of 2600 m/min using a winding machine of a type in which both a spindle and a touch roll were driven to obtain a cheese-shaped package wound with 72 dtex/36 filament fibers.

Thereafter, the fiber wound on the package was drawn to 1.5 times at 30°C, heated with a contact-type hot plate heater at 190°C to shrink the fiber to 0.7 times, and wound up at a speed of 600 m/min to obtain a low-shrinkage polytrimethylene terephthalate fiber (yarn for sheath yarn).

On the other hand, a polyester (polyethylene terephthalate) drawn yarn (total fineness 56 dtex/36 filaments, boiling water shrinkage rate 10%) was prepared as a yarn for core yarn.

Next, the yarn for sheath yarn and the yarn for core yarn were aligned and interlaced at an overfeed rate of 1.5% to obtain an air-jet commingled yarn with an entanglement number of 69/m. Physical properties of the obtained polytrimethylene terephthalate fiber are shown in Table 1, and physical properties of the commingled yarn are shown in Table 2.

### [Example 2]

After a polymer was produced in the same manner as in Example 1, the obtained polymer was dried by a common method to adjust a water content to 50 ppm, melted at 265°C, and extruded through a dual-row spinneret having 72 pores with a diameter of 0.23 mm.

After an oil agent was applied to the extruded molten multifilament in the same manner as in Example 1, the solid multifilament was wound around a roll heated to 50°C with a peripheral speed of 2100 m/min, then wound around a roll heated to 80°C so as to be drawn to 1.3 times, and then wound at a winding speed of 2600 m/min using a winding machine of a type in which both a spindle and a touch roll were driven to obtain a cheese-shaped package wound with 72 dtex/72 filament fibers.

Thereafter, the fiber wound on the package was drawn to 1.4 times at 30°C, heated with a contact-type hot plate heater at 190°C to shrink the fiber to 0.75 times, and wound up at a speed of 600 m/min to obtain a low-shrinkage polytrimethylene terephthalate fiber (yarn for sheath yarn).

On the other hand, a polyester (polyethylene terephthalate) drawn yarn (total fineness 56 dtex/36 filaments, boiling water shrinkage rate 13%) was prepared as a yarn for core yarn.

Next, the yarn for sheath yarn and the yarn for core yarn were aligned and interlaced at an overfeed rate of 1.5% in the same manner as in Example 1 to obtain an air-jet commingled yarn with an entanglement number of 71/m. Physical properties of the obtained polytrimethylene terephthalate fiber are shown in Table 1, and physical properties of the commingled yarn are shown in Table 2.

### [Example 3]

After a polymer was prepared in the same manner as in Example 1, the obtained polymer was dried by a common method to adjust a water content to 50 ppm, then melted at 265°C, and extruded through a single-row spinneret having 36 pores with a diameter of 0.27 mm.

After an oil agent was applied to the extruded molten multifilament in the same manner as in Example 1, the solid multifilament was wound around a roll heated to 50°C with a peripheral speed of 2350 m/min, then wound around a roll heated to 80°C so as to be drawn to 1.1 times, and then wound at a winding speed of 2600 m/min using a winding machine of a type in which both a spindle and a touch roll were driven to obtain a cheese-shaped package wound with 72 dtex/36 filament fibers.

Thereafter, the fiber wound on the package was drawn to 1.6 times at 30°C, heated with a contact-type hot plate heater at 190°C to shrink the fiber to 0.65 times, and wound up at a speed of 600 m/min to obtain a low-shrinkage polytrimethylene terephthalate fiber (yarn for sheath yarn).

On the other hand, a conjugate drawn yarn (total fineness 56 dtex/24 filaments, boiling water shrinkage rate 17%) obtained by bonding two components of polyester (polyethylene terephthalate/polyethylene terephthalate) was prepared as a yarn for core yarn.

Next, the yarn for sheath yarn and the yarn for core yarn were aligned and interlaced at an overfeed rate of 1.5% in the same manner as in Example 1 to obtain an air-jet commingled yarn with an entanglement number of 65/m. Physical properties of the obtained polytrimethylene terephthalate fiber are shown in Table 1, and physical properties of the commingled yarn are shown in Table 2.

### [Example 4]

After a polymer was prepared in the same manner as in Example 1, the obtained polymer was dried by a common method to adjust a water content to 50 ppm, and melted at 265°C, and extruded through a single-row spinneret having 36 pores with a diameter of 0.27 mm.

After an oil agent was applied to the extruded molten multifilament in the same manner as in Example 1, the solid multifilament was wound around a roll heated to 50°C with a peripheral speed of 3000 m/min, then wound around a roll heated to 80°C so as to be drawn to 1.2 times, and then wound at a winding speed of 3600 m/min using a winding machine of a type in which both a spindle and a touch roll were driven to obtain a cheese-shaped package wound with 56 dtex/36 filament fibers.

Thereafter, the fiber wound on the package was drawn to 1.3 times at 30°C, heated with a contact-type hot plate heater at 190°C to shrink the fiber to 0.85 times, and wound up at a speed of 600 m/min to obtain a low-shrinkage polytrimethylene terephthalate fiber (yarn for sheath yarn).

On the other hand, a conjugate drawn yarn (total fineness 33 dtex/24 filaments, boiling water shrinkage rate 21%) obtained by bonding polyethylene terephthalate and polytrimethylene terephthalate was prepared as a yarn for core yarn.

Next, the sheath yarn and the core yarn were aligned and interlaced at an overfeed rate of 1.5% in the same manner as in Example 1 to obtain an air-jet commingled yarn with an entanglement number of 71/m. Physical properties of the obtained polytrimethylene terephthalate fiber are shown in Table 1, and physical properties of the commingled yarn are shown in Table 2.

### [Examples 5 and 6]

The same procedure as in Example 1 was performed except that a cross-sectional shape of a sheath yarn and the number of single fibers in Example 1 were changed as shown in Table 1. Physical properties of the obtained polytrimethylene terephthalate fiber are shown in Table 1, and physical properties of the commingled yarn are shown in Table 2.

### [Comparative Example 1]

After a polymer was prepared in the same manner as in Example 1, the obtained polymer was dried by a common method to adjust a water content to 50 ppm, then melted at 265°C, and extruded through a single-row spinneret having 36 pores with a diameter of 0.27 mm.

After an oil agent was applied to the extruded molten multifilament by the same method as in Example 1, the solid multifilament was wound around a roll heated to 55°C with a peripheral speed of 1500 m/min, then wound around a roll heated to 130°C so as to be drawn to 2.1 times, and then wound at a winding speed of 3000 m/min using a winding machine of a type in which both a spindle and a touch roll were driven to obtain a cheese-shaped package wound with 72 dtex/36 filament fibers (polytrimethylene terephthalate fiber yarns for sheath yarn).

On the other hand, a polyester (polyethylene terephthalate) drawn yarn (total fineness 56 dtex/36 filaments, boiling water shrinkage rate 12%) was prepared as a yarn for core yarn.

Next, the sheath yarn and the core yarn were aligned and interlaced at an overfeed rate of 1.5% in the same manner as in Example 1 to obtain an air-jet commingled yarn with an entanglement number of 65/m. Physical properties of the obtained polytrimethylene terephthalate fiber are shown in Table 1, and physical properties of the commingled yarn are shown in Table 2.

The obtained air-jet commingled yarn had a small core-sheath yarn length difference and was poor in swelling.

### [Comparative Example 2]

After a polymer was prepared in the same manner as in Example 1, the obtained polymer was dried by a common method to adjust a water content to 50 ppm, then melted at 265°C, and extruded through a single-row spinneret having 36 pores with a diameter of 0.27 mm.

After an oil agent was applied to the extruded molten multifilament in the same manner as in Example 1, the solid multifilament was wound around a roll heated to 55°C with a peripheral speed of 1500 m/min, then wound around a roll heated to 130°C so as to be drawn to 2.1 times, and then wound at a winding speed of 3000 m/min using a winding machine of a type in which both a spindle and a touch roll were driven to obtain a cheese-shaped package wound with 56 dtex/36 filament fibers.

Thereafter, the fiber wound on the package was drawn to 1.05 times at 30°C, heated with a contact-type hot plate heater at 190°C to shrink the fiber to 0.92 times, and wound up at a speed of 600 m/min to obtain a tritrimethylene terephthalate fiber (yarn for sheath yarn).

On the other hand, a polyester (polyethylene terephthalate) drawn yarn (total fineness 56 dtex/36 yarns, boiling water shrinkage rate 10%) was prepared as a yarn for core yarn.

Next, the yarn for sheath yarn and the yarn for core yarn were aligned and interlaced at an overfeed rate of 1.5% in the same manner as in Example 1 to obtain an air-jet commingled yarn with an entanglement number of 63/m. Physical properties of the obtained polytrimethylene terephthalate fiber are shown in Table 1, and physical properties of the commingled yarn are shown in Table 2.

The obtained air-jet commingled yarn had a stiff sheath yarn and was poor in hand.

**[Table 1]**

| | Sheath yarn (low-shrinkage PTT yarn) | | | | | | | | | | | | |
|---|---|---|---|---|---|---|---|---|---|---|---|---|---|
| | Total fineness dtex | Number of single fibers filament | Cross-sectional shape | Intrinsic viscosity dl/g | Glass transition point °C | Boiling water shrinkage rate BWS% | Breaking strength cN/dtex | Breaking elongation % | Modulus at elongation of 20% cN/dtex | Specific gravity | Birefringence | Temperature at which thermal stress maximum value is present °C | Thermal stress maximum value cN/dtex |
| Example 1 | 69 | 36 | Round | 1.00 | 51 | 2 | 2.4 | 70 | 1.5 | 1.333 | 0.055 | 69 | 0.07 |
| Example 2 | 69 | 72 | Round | 1.00 | 51 | 3 | 2.5 | 65 | 1.7 | 1.334 | 0.057 | 69 | 0.07 |
| Example 3 | 69 | 36 | Round | 1.00 | 51 | 2 | 2.3 | 70 | 1.2 | 1.332 | 0.052 | 68 | 0.06 |
| Example 4 | 51 | 36 | Round | 1.00 | 51 | 4 | 2.7 | 55 | 2.3 | 1.322 | 0.064 | 69 | 0.07 |
| Example 5 | 69 | 36 | Cross | 1.00 | 51 | 2 | 2.4 | 72 | 1.5 | 1.333 | 0.055 | 68 | 0.065 |
| Example 6 | 69 | 72 | Triangular | 1.00 | 51 | 3 | 2.5 | 62 | 1.7 | 1.333 | 0.056 | 68 | 0.07 |
| Comparative Example 1 | 56 | 36 | Round | 1.00 | 51 | 7 | 2.7 | 40 | 6.0 | 1.345 | 0.062 | 180 | 0.30 |
| Comparative Example 2 | 64 | 36 | Round | 1.00 | 51 | 3 | 2.9 | 60 | 6.5 | 1.369 | 0.049 | 200 | 0.09 |

**[Table 2]**

| | Air-jet commingled yarn | | | | | | |
|---|---|---|---|---|---|---|---|
| | Total fineness dtex | Number of single fibers filament | Breaking strength cN/dtex | Breaking elongation % | Number of entanglements piece/m | Yarn length difference % | Hand |
| Example 1 | 131 | 72 | 2.7 | 23 | 69 | 8 | A |
| Example 2 | 130 | 108 | 2.5 | 25 | 71 | 10 | A |
| Example 3 | 134 | 60 | 2.3 | 28 | 65 | 15 | A |
| Example 4 | 90 | 60 | 2.2 | 29 | 71 | 17 | A |
| Example 5 | 131 | 72 | 2.7 | 23 | 69 | 8 | A |
| Example 6 | 130 | 108 | 2.5 | 25 | 71 | 9 | A |
| Comparative Example 1 | 130 | 72 | 2.8 | 22 | 65 | 5 | C |
| Comparative Example 2 | 92 | 60 | 2.9 | 24 | 63 | 7 | C |

### Description of Embodiments

### Industrial Applicability

According to the present invention, a low-shrinkage fiber substantially composed of polytrimethylene terephthalate, which can be used to produce a raw yarn for cloth having a small shrinkage rate on heating and a soft hand, and a method for producing the same, an air-jet commingled yarn containing the polytrimethylene terephthalate fiber, and cloth composed thereof can be provided, and therefore, the industrial value thereof is extremely high.

## Claims

1. A polytrimethylene terephthalate fiber comprising:
90 mol% or more of a trimethylene terephthalate repeating unit, wherein
the polytrimethylene terephthalate fiber has a boiling water shrinkage rate of 5% or less and a modulus at an elongation of 20% of 5 cN/dtex or less.

2. The polytrimethylene terephthalate fiber according to claim 1, wherein
the polytrimethylene terephthalate fiber has a birefringence Δn of 0.040 or more and a specific gravity of 1.350 or less.

3. The polytrimethylene terephthalate fiber according to claim 1 or 2, wherein
the polytrimethylene terephthalate fiber has a thermal stress peak at 50°C to 100°C and a thermal stress peak value of 0.2 cN/dtex or less.

4. The polytrimethylene terephthalate fiber according to claim 1 or 2, wherein
the polytrimethylene terephthalate fiber has breaking strength of 1.5 cN/dtex to 3.5 cN/dtex and a breaking elongation of 30% to 100%.

5. A method for producing a polytrimethylene terephthalate fiber, the method comprising:
melting and solidifying polytrimethylene terephthalate composed of 90 mol% or more of a trimethylene terephthalate repeating unit;
winding up the polytrimethylene terephthalate at a winding speed of 1000 m/min or more;
drawing the polytrimethylene terephthalate to 1.1 times or more at a temperature equal to or lower than a glass transition point of the polytrimethylene terephthalate; and
shrinking the fiber at a ratio of 0.5 times to 0.9 times while heating.

6. An air-jet commingled yarn comprising:
the polytrimethylene terephthalate fiber according to any one of claims 1 to 4; and
a polyester fiber.

7. The air-jet commingled yarn according to claim 6, wherein
the polyester fiber has a boiling water shrinkage rate of 7% to 50%.

8. The air-jet commingled yarn according to claim 6 or 7, further comprising:
a modified cross-section fiber.

9. A core-sheath type air-jet commingled yarn obtained by heat-treating the air-jet commingled yarn according to claim 6, the core-sheath type air-jet commingled yarn comprising:
a core yarn; and
a sheath yarn, wherein
the air-jet commingled yarn has a total fineness of 30 dtex to 400 dtex,
the core yarn is composed of a polyester fiber,
the sheath yarn is composed of a polytrimethylene terephthalate fiber having a single fiber fineness of 0.3 dtex to 10 dtex, and
a yarn length difference between the core yarn and the sheath yarn is 5% or more, as defined by the following method,
(method for measuring yarn length difference)
the core-sheath type air-jet commingled yarn is treated in boiling water, then cut to a length of 5 cm under a load of 0.1 cN (0.098 g) × total fineness (dtex) of the core-sheath type air-jet commingled yarn, a polyester fiber A (single fiber) and a polytrimethylene terephthalate fiber B (single fiber) are taken out from the cut core-sheath type air-jet commingled yarn, a length of each is measured under a load of 0.1 cN (0.098 g) × single fiber fineness (dtex) thereof, and the yarn length difference (%) is calculated by the following formula:$Yarn length difference \left(%\right) = \left(LB - LA\right) / LA \times 100$
where LA is a yarn length (cm) of the polyester fiber of the core yarn, and LB is a yarn length (cm) of the polytrimethylene terephthalate fiber of the sheath yarn.

10. The core-sheath type air-jet commingled yarn according to claim 9, wherein
a weight ratio of the sheath yarn to a total weight of the core-sheath type air-jet commingled yarn is 50% to 90%.

11. The core-sheath type air-jet commingled yarn according to claim 9 or 10, further comprising:
a modified cross-section fiber.

12. Cloth comprising:
the air-jet commingled yarn according to any one of claims 6 to 8.

13. Cloth comprising:
the core-sheath type air-jet commingled yarn according to any one of claims 9 to 11.
